

## UNITED STATES PATENT OFFICE.

BERT A. STAGNER, OF LONG BEACH, CALIFORNIA.

MOTHPROOF FELT, ETC.

No Drawing.

Application filed November 22, 1923. Serial No. 676,284.

*To all whom it may concern:*

Be it known that I, BERT A. STAGNER, a citizen of the United States, residing at Long Beach, in the county of Los Angeles, 5 State of California, have invented certain new and useful Improvements in Mothproof Felt, Etc.; and I do hereby declare the following to be a full, clear, and exact description of the invention, such as will enable 10 others skilled in the art to which it appertains to make and use the same.

This invention relates to felted hair products and the like, and has among its principal objects the provision of a hair felt 15 pad, particularly adapted for use as a buffer beneath rugs, which is more satisfactory and more resistant toward deteriorating influences than the felted hair pads hitherto known.

20 It frequently happens under certain circumstances that hair felt pads or mattings, for use beneath rugs and carpets as a buffer to protect them from wear and to add resilience to the floor covering, become infested with clothes moth, carpet beetle, larvae, etc. The effect of such infestation is to deteriorate or destroy the pad or floor covering besides creating a nuisance. The methods hitherto commonly employed for 25 overcoming these objectionable features are very difficult to apply or else they are ineffective and frequently produce deteriorating effects upon the floor covering. Also, they frequently add to the fire hazard 30 involved, as for example, when petroleum oils or the like are employed as the disinfecting agent.

The present invention includes an improved felted hair product which is vermin 40 proof and which at the same time possesses substantially all the inherent advantages of normal hair felt as a buffer and for other similar uses and which furthermore retains these desirable properties unimpaired for the 45 ordinary life of the felt. The present invention also includes an improved disinfecting agent or solution, and an improved method of applying the same to a wide variety of products made from hair, but 50 more particularly to the treatment of felted hair products to be used as buffers beneath floor coverings.

I have found that the proofing of hair felt and the like against vermin may be most satisfactorily accomplished by means of a

disinfecting agent which is free from odor and which does not dust off or become removed by vacuum sweepers and which does not, in general, lose its potency with age under the peculiar conditions of use or 60 storage to which such pads or felts are ordinarily subjected. I have also found that it is highly desirable that a proofing agent for the above purposes shall be of such nature that it will readily penetrate 65 the fibres of the hair or felt or pad to a uniform extent throughout the material so as to subject each portion and fibre thereof to the disinfecting agent as otherwise I have found that the vermin will attack the 70 material at points which have not been subjected to the treatment and will there form nesting places or operating places for the larvae. The attack of the vermin will then sometimes spread from these nesting places 75 to the floor covering and even to other portions of the incompletely treated hair itself.

I have discovered that a solution of ordinary white arsenic in alkali or soda solution when applied in accordance with the method 80 of my invention fulfills the requirements that I have found to be necessary for good results as already mentioned, and at the same time this solution is free from the objections of the disinfecting agents hitherto used 85 for this purpose, and when applied it is particularly effective against moth and beetle larvae and the like.

I have also discovered that sodium arsenite solution as ordinarily prepared is not so 90 satisfactory as the modified solution of this invention for treating such felted hair products, mattings and the like, and particularly for treating closely woven  $\frac{1}{4}$ " to  $\frac{3}{4}$ " hair felt pads such as are used under carpets and rugs and the like. I have found that this less satisfactory effect of ordinary sodium arsenite solution is due, in part at least, to its failure to penetrate each and every part of the felt, and I believe this 100 failure to thus penetrate the felt and to cover each hair fibre with the disinfecting agent is due to the effect of an oil film normally present on hair fibres which is of such nature that a high interfacial tension 105 between the oil film and the aqueous solution is produced so that the felt is effectively water proofed, so to speak, against the solution causing the felt to resist the penetration of the solution into the pores of the 110

felt and also preventing the wetting of the hair fibres by the solution. Moreover, I have found that if the water solution of ordinary sodium arsenite be mechanically 5 forced into the felt, as by the application of very high pressure, the arsenite, even so, when dried will readily dust out under the conditions of ordinary use and thus leave the felt unprotected.

10 The present invention further includes the application of an improved arsenite solution to the hair felt and the subsequent removal of the water therefrom, preferably by ordinary drying. The finished disinfested 15 felt is substantially unaffected by this treatment so far as retention of its desirable properties is concerned, and furthermore, the residue of the disinfesting agent left in the felt does not readily dust off from the fibres 20 but adheres tenaciously thereto so that it is not removed to any objectionable extent in use or by the action of vacuum sweepers and the like. Furthermore, in the application of my improved solution to the fabric, no 25 complicated means of forcing the solution into the pores of the felt is necessary, but on the contrary, the improved solution penetrates readily and easily into the felt wetting uniformly all the fibres thereof, and advan- 30 tageously may be applied to the felt by atomizing or spraying it thereon.

My improved arsenical solution comprises preferably a soluble alkali arsenite containing animal glue, or other similar glue, and a 35 soluble agent, such as ordinary soap or sodium oleate, capable of substantially reducing the surface tension of the solution. My invention further includes the addition of such quantity of the soap or equivalent 40 agent to the solution as will reduce the surface tension thereof to that range which will impart the desired penetrating properties to the solution without at the same time adversely affecting the adhesive power of the 45 solution after drying, or without attenuating the arsenic content of the dried solution to an objectionable degree or producing any other deleterious effects, either during the application of the solution or afterwards.

50 The enormously enhanced wetting power of my disinfesting solution can be effectively demonstrated by pouring a little of the ordinary soapless arsenite solution upon a small piece of the hair felt and then comparing its 55 behaviour with my improved arsenite solution containing the soap. In the first case the soapless solution will stand for a protracted period on the felt without sinking into or wetting it, but in the second case the 60 soap-containing solution wets and sinks into the felt promptly and if a considerable excess of the solution be added to the hair felt the solution passes through the felt with almost as great ease as water passes through 65 an ordinary sieve.

My improved disinfesting solution is more readily atomized or broken up into spray than similar solutions hitherto in use in this art and the smaller droplets thus produced by spraying or atomizing also contribute to 70 a more uniform distribution throughout the felt and over the surface of the fibres when applied in this manner.

In the practice of my invention, I may apply my improved solution to the felt by 75 spraying it upon the hair fibre either before or during the felting operation or while the felt is being passed on conveyers on its way to the final drying closets in the process of manufacturing, as ordinarily carried out, 80 but I find it particularly advantageous to apply the solution during the felting operation, since in the usual process of manufacture it is usually necessary that the fibre be heavily moistened with water in order to 85 aid in the proper felting of the fibres.

I have found that a satisfactory disinfesting solution for proofing hair felt against moth, beetle larvae and the like may be prepared by mixing certain ingredients in cer- 90 tain proportions as shown in the following formula, which is given by way of an example or embodiment of my improved disinfesting solution, it being understood that my invention is illustrated thereby and is 95 not restricted to the particular ingredients or to the particular proportions described.

Water, 10 gallons; soda ash crystals, 43 pounds; white arsenic, 10 pounds; glue, 1 100 pound; soap,  $\frac{1}{4}$  to  $\frac{1}{2}$  pound.

The water may be heated to near boiling in an iron mixing kettle, the soda added, and the remaining ingredients then dissolved. About 18.8 pounds of anhydrous soda may be employed in the above formula in place 105 of the soda ash crystals. The soap employed may be, for example, sodium oleate. In place of glue, other suitable adhesives may be employed.

It is to be understood that in the above 110 formula the proportion of water can be varied within rather wide limits but, in general, it is advantageous to employ a sufficient quantity to carry the arsenite, glue and soap 115 throughout the felt and yet less than an amount which would cause objectionable expense in the final drying of the felt due to the larger proportion of water to be evaporated. Likewise, the amount of soap may be varied, but I find that the minimum 120 amount desirable is that which causes the spray droplets to be smaller in size, and more important still, that amount which causes the droplets to sink at once into the felt rather than to stand out on top of the 125 felt as do the ordinary solutions. The glue is preferably a good grade animal glue free from odor and of a quality which does not become brittle when dry. I may, however, substitute for animal glue other glue having 130

similar properties when applied in the manner and in accordance with the method of the present invention, such for example as a properly prepared vegetable or starch glue 5 of the kind known in the textile art as appetarate.

While I have described my invention particularly with reference to the application of arsenite solutions to hair felt, especially 10 adapted for use beneath rugs, it will be apparent that the invention may also be employed in disinfecting and vermin proofing other manufactured hair products, in the treatment of hair products with other arsenic containing solutions, and generally to 15 the treatment of hair products with solutions of disinfecting agents which will not thoroughly wet the hair fibres.

I claim:

- 20 1. The method of disinfecting and proofing manufactured hair products against vermin, which comprises subjecting the fibers of the hair to the action of a solution of an arsenical compound, soap and an adhesive 25 to thoroughly wet the fibers and then allowing the hair product to dry whereby a coating of said compound will be left on the fibers of the hair.
- 20 2. The method of disinfecting and proofing manufactured hair products against vermin, which comprises subjecting the fibers of the hair to the action of a solution of an arsenical compound, an adhesive and a surface tension reducing agent to thoroughly 35 wet the fibers, and then allowing the hair product to dry, whereby a coating of said

compound will be left on the fibers of the hair.

3. As a new article of manufacture, a manufactured hair product impregnated 40 with a solution containing an arsenical compound, soap and adhesive, and having a coating of said solution adhering to the fibers thereof.

4. As a new article of manufacture, a hair 45 product impregnated with a solution containing an arsenical compound, a surface tension reducing agent and an adhesive, and having a coating of said solution adhering to the fibers thereof.

5. As a new product for disinfecting and proofing manufactured hair products against vermin, a solution containing an arsenical compound, a surface tension reducing agent 50 and an adhesive, said solution being adapted to leave an adhering coating thereof on the fibers of the hair.

6. As a new product for disinfecting and proofing manufactured hair products against vermin, a solution containing an arsenical 60 compound, soap and an adhesive, said solution being adapted to leave an adhering coating thereof on the fibers of the hair.

7. The method of applying an arsenic solution to felted hair products which comprises reducing the surface tension of the solution, atomizing the solution into a spray of very fine droplets, and subjecting the felted fibres to the action of the said spray.

In testimony whereof I affix my signature.

BERT A. STAGNER.